

## UNITED STATES PATENT OFFICE

2,526,999

## CADMIUM PLATING BATH

Myron B. Diggin, Matawan, and Otto Kardos, Leonardo, N. J., assignors to Hanson-Van Winkle-Munning Company, Matawan, N. J., a corporation of New Jersey

No Drawing, Application June 7, 1947,  
Serial No. 753,370

2 Claims. (Cl. 204—50)

1

Our invention relates to alkali-cyanide cadmium plating baths, and more particularly to improvements in the composition and performance of such baths.

Important objects of the invention are to improve the character of the deposit and to extend the plating range within which smooth, dense deposits of bright or brilliant surface appearance are obtained.

The objects of the invention are obtained by employing as addition agents in the bath composition one or more oxyheterocyclic compounds containing an oxyheterocyclic ring of 5 or 6 atoms, and hydroxyethyl cellulose, with or without addition of small quantities of nickel salts which are soluble in the cyanide bath. The U. S. patent of Hogaboom & Diggin, No. 1,893,368, patented January 3, 1933, discloses a conventional alkali-cyanide cadmium plating bath to which are added as brighteners various oxyheterocyclic compounds. Such baths may be improved, in accordance with our invention, by adding about 0.025 to 0.2 gm./l. (preferably 0.1 gm./l.), hydroxyethyl cellulose powder, or equivalent amount of solution, and preferably also small quantities of soluble nickel salts.

Conventional cadmium plating baths of the alkali-cyanide type usually contain the following:

|                      |                 |
|----------------------|-----------------|
| Cadmium metal        | 2.0—4.5 oz.     |
| Total sodium cyanide | 8.5—17.5 oz.    |
| Sodium hydroxide     | 1.0—3.2 oz.     |
| Sodium carbonate     | varying amounts |
| Water to make        | 1 gal.          |

The following experiments were performed in Hull Cells (250 ml.) on sheet steel cathodes, at a total current of 1 ampere, 10 minutes plating time, room temperature and with an aqueous bath made up as follows:

|                |          |      |
|----------------|----------|------|
| Cadmium oxide  | Oz./gal. | 3.5  |
| Sodium cyanide |          | 14.5 |

**Example 1.**—To 1 liter of the cadmium plating bath add 12 cc. of furfuryl alcohol (refined) and 0.6 gram nickel sulphate. The Hull Cell plate shows only a whitish semi-brightness from about 10. amps./sq. ft. upwards. The addition of 10 cc./l. of a 1% solution of hydroxyethyl cellulose improved the appearance of the Hull Cell plate in the low current density range and changed the semi-brightness of the plate to a slightly streaky brilliance from 10 to about 35 amps./sq. ft. under the same operating conditions.

**Example 2.**—16 cc. of tetrahydrofurfuryl alcohol and 0.4 gram of nickel sulphate added to 1 liter of the cadmium plating bath give only a semi-bright electrodeposit from about 15 amps./sq. ft. upwards. The further addition of 10 cc./l. of a 1% solution of hydroxyethyl cellulose improves the semi-brightness to brilliance from about 15 to 40 amps./sq. ft. and increases also the brightness in the current density range below 15 amps./sq. ft.

**Example 3.**—The addition of 20 grams furyl acrylate and 0.6 gram nickel sulphate to 1 liter of the cadmium plating bath gives milky, semi-bright deposits over a large current density range. Addition of 10 cc./l. of a 1% solution of hydroxyethyl cellulose improves the semi-brightness to brilliance at about 20 to 30 amps./sq. ft.

**Example 4.**—The addition of 10 cc./l. of a 1% solution of hydroxyethyl cellulose to a conventional cadmium plating bath containing 4 gms./l. hematein (from logwood extract) and 0.6 gm./l. nickel sulphate slightly increases the brightness of the deposit.

**Example 5.**—The addition of 10 cc. of a 1% solution of hydroxyethyl cellulose to 1 liter of a cadmium plating bath containing 2 grams furoin and 0.6 gram of nickel sulphate increases the brilliance of the deposit and extends the current density range for bright deposits.

**Example 6.**—Addition of 10 cc. of a 1% solution of hydroxyethyl cellulose to a cadmium bath containing 1 gm./l. furyl nitroethylene improves noticeably the brightness of the Hull Cell plate.

**Example 7.**—The addition of 10 cc./l. of a 1% solution of hydroxyethyl cellulose to a cadmium plating bath containing 16 c./l. furfurylamine and 0.6 gm./l. nickel sulphate improves the bright quality of the plate and extends the current density range for securing bright deposits.

**Example 8.**—A cadmium plating bath, having added thereto 7.5 to 11.25 gms./l. of caustic alkali-furfural resin and 0.6 gm./l. nickel sulphate, gives semi-bright deposits from 15 amps./sq. ft. upward. The addition of 10 cc./l. of a 1% solution of hydroxyethyl cellulose gives a deposit of high brilliance.

Addition of hydroxyethyl cellulose to a cadmium bath containing only 7.5 to 11.5 gms./l. of caustic alkali-furfural resin but no nickel sulphate gives a noticeable increase in brightness. However, the best results are obtained from baths containing all three addition agents.

Numerous plating tests have shown that the addition of 10 c. c./l. of a 1% solution of hydroxyethyl cellulose, or 0.1 gm./l. of the solid

hydroxyethyl cellulose, to conventional cadmium plating baths containing caustic alkali-furfural resin (preferably 7.5 to 11.25 gms./l.) and nickel (preferably 0.09 to 0.27 gm./l. of nickel metal) added in the form of the sulphate, carbonate, formate, cyanide, complex cyanide or the like, will give electrodeposits of improved brightness at current densities ranging from 15 to 40 amps./sq. ft. A barrel plating cadmium solution containing 7.5 to 11.25 gms./l. caustic alkali-furfural resin, with or without nickel salts, can be made to produce a noticeably brighter deposit by the addition of hydroxyethyl cellulose.

The caustic alkali-furfural resin can be prepared, for example, by slowly adding 15 pounds of sodium hydroxide, dissolved in 30 pounds of water, to 67.5 pounds furfural while cooling and stirring, and then evaporating the reaction mixture to dryness under vacuum.

*Example 9.*—Brilliant deposits are obtained from cadmium solutions containing small quantities of a high-boiling distillation residue, obtained as a by-product in the manufacture of tetrahydrofurfuryl alcohol, and furthermore hydroxyethyl cellulose and nickel salts. This distillation residue is a dark liquid of moderate viscosity, a large part of which cannot be distilled at 6 mm. pressure. It contains considerable amounts of oxyheterocyclic condensation products, as on treatment with phosphoric acid considerable amounts of tetrahydrofurfuryl alcohol are obtained. The addition of 3 grams of this residue and 0.6 gram of nickel sulphate to 1 liter of the cadmium plating bath gives a small bright plating range at about 35 amps./sq. ft. in the Hull Cell, and the further addition of 10 c. c. of hydroxyethyl cellulose (1% solution) widens the bright plating current density range considerably.

*Example 10.*—100 grams of the distillation residue of tetrahydrofurfuryl alcohol, above described, are mixed with water to make 400 c. c. of solution. The resulting very turbid solution is treated with enough activated carbon (Darco S-51) to give a clear filtrate. The addition of 16 c. c. of this clear solution, corresponding to 4 grams of crude distillation residue, and 0.6 gram of nickel sulphate to 1 liter of the cadmium plating bath gives a solution from which a semi-bright deposit is obtained at about 15 amps./sq. ft., which increases in brightness as the current density is raised until it becomes brilliant at about 40 amps./sq. ft. On the addition of 10 c. c. of a 1% solution of hydroxyethyl cellulose to this bath, a brilliant deposit is obtained from about 10 amps./sq. ft. to about 40 amps./sq. ft.

*Example 11.*—As a further example of the effect of adding hydroxyethyl cellulose to an alkali-cyanide cadmium plating bath containing oxyheterocyclic addition agents, we may refer

to such baths in which the oxyheterocyclic compound is in the form of acids formed by "Autoxidation of Furfural" as described by Dunlop, Stout and Swadesh in "Industrial and Engineering Chemistry," vol. 38, pages 705 to 708, July 1946, under the name of Solid-Indicator acids. On addition of 2 to 4 gms./l. of said acids (brown powder) and of 0.6 gm./l. of nickel sulphate to a cadmium plating bath, a bright cadmium deposit is obtainable within a small range of rather high current density. The addition of 10 c. c./l. of a 1% solution of hydroxyethyl cellulose considerably increases the brightness of the deposit and also considerably extends the range of current density under which the brightness occurs.

It may be mentioned that hydroxyethyl cellulose seems to be quite stable in cyanide cadmium solutions, and that only relatively small replenishments need to be made from time to time.

We claim:

1. An alkali-cyanide cadmium plating bath containing in solution as addition agents an oxyheterocyclic compound selected from the group consisting of furfuryl alcohol, tetrahydrofurfuryl alcohol, alkali furyl acrylate, furoin, furyl nitroethylene, and a bath-soluble caustic alkali-furfural resin, in amounts from about 1 to 20 gms./l., and said cyanide cadmium bath also containing in solution 0.025 to 0.2 gm./l. hydroxyethyl cellulose.

2. An alkali-cyanide cadmium plating bath containing in solution as addition agents a bath-soluble nickel salt in amounts substantially equivalent to 0.09 to 0.27 gm./l. of nickel, and an oxyheterocyclic compound selected from the group consisting of furfuryl alcohol, tetrahydrofurfuryl alcohol, alkali furyl acrylate, furoin, furyl nitroethylene, and a bath-soluble caustic alkali-furfural resin, in amounts from about 1 to 20 gms./l., and said cyanide cadmium bath also containing in solution 0.025 to 0.2 gm./l. hydroxyethyl cellulose.

MYRON B. DIGGIN,  
OTTO KARDOS.

#### REFERENCES CITED

The following references are of record in the file of this patent:

#### UNITED STATES PATENTS

| Number    | Name             | Date          |
|-----------|------------------|---------------|
| 1,681,509 | Westbrook        | Aug. 21, 1928 |
| 1,893,368 | Hogaboom         | Jan. 3, 1933  |
| 2,107,806 | Soderberg et al. | Feb. 8, 1938  |

#### FOREIGN PATENTS

| Number  | Country | Date          |
|---------|---------|---------------|
| 704,989 | Germany | Apr. 17, 1941 |

#### OTHER REFERENCES

Transactions of the American Electrochemical Society, preprint 80-27 (1941), pages 335-340.